

Oct. 25, 1938.

N. BRACKETT

2,134,324

DRY GRAPHITE LUBRICATED FABRIC PACKING

Filed Dec. 14, 1937



Witness:

Chas. E. Marsh, Chritton, Miles, Davies, Hirsch & Dawson & Atteys.

Inventor  
Newell Brackett

## UNITED STATES PATENT OFFICE

2,134,324

DRY GRAPHITE LUBRICATED FABRIC  
PACKING

Newell Brackett, Philadelphia, Pa.

Application December 14, 1937, Serial No. 179,762

## 4 Claims. (Cl. 96—26)

This invention relates to improvements in packing and more particularly to what may be called dry-graphite lubricated and metalized fabric and semi-metallic fabric packing.

5 Conventional fabric packings or semi-metallic fabric packings, as used commercially, generally consist of certain fabric fibers such as flax, jute, cotton, asbestos and others, spun; twisted or wrapped into rovings and yarns that are braided, 10 twisted or woven into packings of various sizes for piston rods, plungers, shafts, valve stems or other moving, mechanical parts. Such packings are impregnated with liquid lubricants, greases and lubricating compounds to reduce friction. 15 Said packings, furthermore, are frequently armored or combined with various metals such as lead, copper, aluminum, etc., to further reduce friction and give a full metallic or semi-metallic wearing face on the moving parts. The method 20 for combining the metal with the other ingredients usually involves a process of wrapping, twisting, or interbraiding the metal in the form of foil or wire, to produce the metallic or semi-metallic wearing face.

25 The objection to such packings is that the greases or other lubricating compounds will, under certain conditions and low temperatures, soften or melt and run out or be squeezed out of the packing under compression and under 30 continued wear. Thus the packing does not retain its original characteristics and after a certain interval becomes unsuited for its purpose.

One object of the present invention is to provide an improved method and the product resulting therefrom, in which more or less of an anti-friction metal and a dry lubricant are introduced into a packing, which lubricant will not melt, squeeze out or be forced out under compression and continued use.

40 In carrying out the invention the packing is impregnated with graphite and anti-friction metal in finely divided form, together with a suitable binder. A small strand is used, preferably of flax, although jute, cotton, asbestos fiber 45 and other suitable fabrics may be used.

As contributory to the general object, therefore, the invention has as a further object, the provision of a packing made up of flax strands or yarn or other fibrous strands, each of which is 50 thoroughly coated and more or less impregnated with graphite and powdered metal. Due to the small diameter of the strands, the amount of graphite and metal in the packing may be considerably greater than would be the case with 55 strands of larger diameter, and, furthermore,

said graphite and metal is more uniformly distributed throughout the entire packing. In other words, the effect is that of a thorough impregnation of the strands throughout any given cross-section of the product.

5 In manufacturing such fabric packing either by twisting, wrapping, braiding or weaving, the pulverized metal that is used may be sprayed, forced or otherwise applied onto and between the fibers, in combination with a binder which permits the small particles to adhere to said fibers and form a metallic or semi-metallic wearing face in the finished packing. It is another object of the invention to provide an improved product made in this manner.

10 An additional object is to provide in the combination, a suitable binder which may consist of a rubber compound, various types of cement of a compound of such ingredients, preferably one which can be vulcanized and produce a 15 product suitable for use to seal against leakage of water, steam, air, gases, petroleum products, etc.

15 Before describing apparatus suitable for carrying out the process, the latter is outlined briefly as follows. The flax, asbestos, or other strands are drawn off of suitable supports such as reels and have a binder and vulcanizing agent applied thereto, preferably while separated from each other, hereinafter described more in detail. The 20 strands are then run through small particles of anti-friction metal such as lead and graphite i. e. atomized or powdered lead pre-mixed with graphite. Said strands are then preferably twisted to form a single multiple-ply roving after 25 which the same are wound on bobbins and used in a braiding machine to form a braided product. The braiding operation builds up a packing of the desired cross-section, usually square, but in some cases round, after which said packing is 30 then preferably passed through a receptacle, where an additional binder and an extra coating of graphite and powdered metal are applied to the surface. At this point the packing may be run through rollers to square it more accurately, 35 which operation compresses it more or less as may be desired. It is thereafter vulcanized. Following this step it may be given a final die or roller operation to insure an accurate cross-sectional outline. The packing may, if desired, 40 be vulcanized before squaring it through rollers.

45 In the accompanying drawing there is illustrated diagrammatically, apparatus for carrying out the above described process and illustrating also the product in more than one form.

Fig. 1 is a top plan view, somewhat diagrammatic, of devices for successively performing the steps described;

Fig. 2 is an elevation of the same;

5 Fig. 3 is an elevation of a perforated plate;

Fig. 4 is a perspective view of the finished packing in one form;

10 Fig. 5 is a perspective view of a length of said packing coiled for packing and shipment;

15 Fig. 6 is a side elevation of an individual ring or split ring cut from a length of packing and bent to circular form; and

Fig. 7 is a perspective view of a modification.

As shown in Figs. 1 and 2, a suitable rack or frame 11 is provided having a number of reels 12 mounted thereon. There may be anywhere from about ten to thirty-five such reels, although these limits may be varied and the number depends on the product desired. These flax strands or 20 asbestos or other fibrous strands are drawn continuously past guides 13, into and through a container 14 and under a roller 15, the latter being submerged in a suitable binder and vulcanizing agent which is preferably rubber, natural or synthetic, among which may be mentioned the commercial product Neoprene. Said strands are drawn through a receptacle 14 in a separated or spread out arrangement, to insure a thorough impregnation thereof. As the strands leave said receptacle they pass a device for wiping off or removing the surplus binder, as for example rollers 16, constituting a squeegee. Said strands then pass over a guide 17 which keeps them separated, and down into and through a second receptacle 35 18 and under the roller 19 therein. Said receptacle contains a dry lubricant such as graphite and anti-friction metal in finely divided form. For example, the mixture may consist of atomized or powdered lead premixed with 40 graphite. The proportions in one instance might be one part of lead by volume to five parts or less of graphite. More or less lead may be used and in fact the lead content may be reduced or substantially eliminated in some cases, but it is 45 preferable to use some lead as it seems to protect the flax or asbestos from wear, in addition to its other well known advantages as a friction reducing packing ingredient. The preliminary application of the binder causes the graphite and powdered metal to adhere satisfactorily to the 50 strands. The latter, before leaving the receptacle, pass through a perforated plate 20 which evenly spaces the strands in a concentric arrangement whereby they may be later twisted 55 together in an even manner and are then brought together by being passed through an opening 21 in the wall of said receptacle after which they pass through a rotating, twisting device 22. By 60 passing said strands through the perforated plate 20 and the small opening 21, the excess graphite and atomized lead are prevented from being shaken off or thrown off during the twisting operation and the result is that more of these ingredients are incorporated into the braid than would otherwise be the case, and there is more metal on the 65 face of the packing when it is finished. The twisted strands form a single multiple-ply rope, the number depending on the desired size of packing. For example, about fourteen or fifteen 70 flax strands would be twisted together to make each of the composite flax strands used in forming a  $\frac{1}{8}$  inch square flax packing. For a one inch flax packing about thirty-five strands per rope 75 would be used. Said twisted strands, before braiding, have been twisted preferably two or

three turns per foot and half of said strands are twisted in one direction and the other half in the other direction.

From the twisting device, the composite, twisted strands are wound on a suitable bobbin 23. 5 The bobbins are those suitable for use in a braiding machine, indicated diagrammatically at 24. Eight bobbins are ordinarily used in such machines for a square product, in addition to providing a center and four corner cores. Four of 10 the bobbins have the strands on them twisted in one direction and the other four in the opposite direction. The cores are formed by combining together some of the same strands mentioned above or other similar strands. The ropes or 15 strands are braided about the corner cores 25 and the center core 26 in the conventional manner.

After braiding, the binder is again applied in a receptacle 27, similar to the one previously described, and an extra coating of graphite and lead, preferably 50-50 by volume, is applied to the surface in a receptacle 28, similar in general to the one previously described. At this point the packing may be passed between rollers of 25 conventional design (not shown) to square it more accurately or change its cross-sectional dimensions, which step compresses it more or less, after which it is vulcanized in any conventional vulcanizing apparatus 29, using a suitable source 30 of heat 30. The rubber compound used is such as to permit vulcanizing preferably at the lowest possible temperature to prevent possible damage to fibers which char at low temperatures. Maximum heat resistance is also given to the product 35 as well as resistance to the deteriorating effects of oil.

As a final step the packing may be given a die or roller operation to insure accurate dimensions.

40 The product 31 in one form is shown in Fig. 4, the cores 25 and 26 being indicated at the end. The product has a semi-metallic wearing face of anti-frictional properties and the packing as a whole has the advantage of resiliency, the fibers 45 are protected against rotting when in contact with water and other liquids, the lubrication remains in the packing and cannot melt out, wash out or squeeze out, and very slight adjustment is necessary to control the leakage if any exists. It 50 can readily be bent into coils such as shown at 32 in Fig. 5, or cut up and bent into rings 33, as shown in Fig. 6 and installed in the usual manner, although it is preferable and customary to coil braided packings as a flat spiral, known to 55 the trade as a "coil".

A further important advantage is that packing rings when formed of this material return to their original size approximately, when compression thereon is relaxed. For example, where the packing is applied to propeller shafts on ships and on centrifugal pumps in service generally, a certain small leakage is desired to lubricate the packing. On shut downs, as where the ship is docked, leakage can be stopped by gland adjustment. Upon further operation, the glands are slackened off and the desired leakage obtained without adversely affecting the packing.

Where conventional flax packings are used, the lubricants may consist of tallow, Japan wax, 70 paraffin wax, lubricating oils, etc., which melt at low temperatures and run out of the box, making it necessary to adjust the glands to compensate for this loss. Packings thus deficient in lubrication cause unnecessary friction and wear 75

of the shafts, as the fiber itself without lubrication will score the shaft. It is also necessary in certain cases to add additional rings. The improved packing described herein has the further advantage of preventing the fibers from slipping one on the other. Such slipping action would result in the fibers extruding beneath the gland, causing heating, and resulting in a loss of packing material. Although flax and asbestos are the preferred fibrous materials, any suitable fibrous material may be used, i. e. vegetable, (cotton, jute, hemp, etc.) mineral, (spun glass) or animal, i. e. wool.

The packing may be reinforced, if desired, by the use of a suitable, stiff core, to add longitudinal rigidity to it. Also, in the case of commercial asbestos which usually contains a little cotton, the strands are preferably reinforced with fine, non-abrasive wires, particularly where high temperatures and high pressures are to be encountered.

Fig. 7 shows a packing, preferably round in form, which is made by braiding the previously described material on a core 34, which core may be initially a small, round core made of a few strands of treated yarn, or made of non-abrasive metal or other suitable material. One or more concentric jackets 35, 36, may be braided over said core. In this construction also the packing has the dry lubrication and powdered metal distributed substantially uniformly throughout the cross-section thereof. It will be understood also that successive jackets may be braided over a packing having a square cross-section such as shown in Fig. 4. Where these concentric jacket over jacket arrangements are used, the graphite and lead may be omitted from the inner jackets as it is more readily available in the outer jackets. The vulcanizing material not only serves the purpose previously described but tends to insure against slippage of one concentric layer on an-

other, i. e. it tends to prevent slippage of the inner layer with respect to the core, as well as slippage of any outside layers with respect to each other. Where the core is made of a small strip of soft metal such as lead for example, the packing which is braided about the core will, for many purposes adhere thereto sufficiently to prevent slippage. However, when a ring such as 33, shown in Fig. 6, surrounds a rotating shaft there is a tendency for the ring to open and form a gap between its ends. This objectionable tendency may be offset by providing a core such as previously referred to and so constructing the packing that there is no slippage of the packing material with respect to said core.

I claim:

1. A packing comprising small strands of fibrous material, each of which is impregnated with a heat treated binder and also coated and partially impregnated with graphite, said strands being twisted together and intertwined with other twisted strands in the form of an elongated packing lubricated throughout.

2. A packing comprising several strands of fibrous material, twisted together to form strands of small diameter, each of said strands having a binder which holds a filling of powdered metal and dry lubricant interspersed throughout said packing, whereby the latter has an anti-friction, metalized face, is flexible and resilient, and retains its lubricant despite compression and wear.

3. A packing as in the preceding claim in which the said strands are twisted together to form threads and a plurality of said threads are then braided to a square cross-section.

4. A packing as in claim 1 in which the binder is a vulcanized rubber compound and in which the elongated packing has an additional outer coating of finely divided metal and a dry-lubricant applied thereto.

NEWELL BRACKETT.